

P. M. HAMLIN.

COMPOSITE FIBER AND PROCESS OF MAKING THE SAME.

APPLICATION FILED MAY 25, 1907.

931,865.

Patented Aug. 24, 1909.



Witnesses:

L. Lee.

J. Greenbaum

Inventor:

Pulaski M. Hamlin,  
per Thomas S. Crane, Atty.

# UNITED STATES PATENT OFFICE.

PULASKI M. HAMLIN, OF CATAWISSA, PENNSYLVANIA, ASSIGNOR OF ONE-HALF TO CHARLES H. UNVERZAGT, OF NEW YORK, N. Y.

## COMPOSITE FIBER AND PROCESS OF MAKING THE SAME.

931,865.

Specification of Letters Patent. Patented Aug. 24, 1909.

Application filed May 25, 1907. Serial No. 375,567.

To all whom it may concern:

Be it known that I, PULASKI M. HAMLIN, a citizen of the United States, residing at Shuman street, Catawissa, county of Columbia and State of Pennsylvania, have invented certain new and useful Improvements in Composite Fiber and Processes of Making the Same, fully described and represented in the following specification and the accompanying drawings, forming a part of the same.

The present invention consists of a composite fiber and the process of manufacturing the same.

15 The fiber embodies wood cellulose and straw cellulose incorporated together when first reduced from the wood and straw, so as to produce a fiber of composite nature having a substance of homogeneous character.

20 The object of the invention is to produce a fiber having the qualities of both wood and straw cellulose, but possessing characteristics very different from, and superior to any mere mixture made from previously manufactured wood and straw cellulose.

25 The incorporation of the two fibers is effected in a manner which avoids the use of a beating engine to intimately mingle the fibers, the two fibers being mingled while in a heated condition immediately upon their extraction from the raw materials. This is effected by reducing the fibers simultaneously in separate digesting vessels by any suitable chemical treatment, and commingling the resulting fibers by blowing the contents of the digesters into contact with one another in a suitable blow-tank. The fibers are thus combined while mingled with the 30 chemical liquor required in the digesting process, and while they are still in a heated condition, which greatly softens the fibers and adapts them to commingle and interlace in a manner which can never be effected

35 after they have cooled and the liquor has been washed from them. The amalgamation of the fibers is greatly facilitated by the expansion or explosion of the steam in the tissues. The product thus obtained is not a 40 mixture of fibers, but is a composite fiber of unbleached character, which is readily distinguished by its characteristics from any

mere mixture of previously finished and bleached fibers.

The product is not claimed in the present 55 application, but only the process for producing it.

50 Pine and analogous woods are largely employed for the manufacture of wood cellulose; but it is a well known fact that the cellulose obtained from pine and other analogous woods, while possessing considerable strength, is unsatisfactory for the manufacture of strong fine papers until subsequently treated in the refining engine.

55 The process employed for making wood fiber from pine or other analogous woods produces a pulp of soft spongy character and uneven appearance, technically known as "mottled," and this appearance can only be corrected by treating the fiber in beating and refining engines for a sufficient time to 60 make the fiber smooth and uniform in appearance.

65 The chemical treatment employed in reducing the wood produces a long fiber; but the treatment required to make the fiber smooth tends to shorten the fiber, and is in any case detrimental to the strength of the 70 paper made from such wood fibers.

75 One object of this invention is to utilize the long fiber of wood without treating it in a beating engine, and thus avoid the shortening and weakening of the fiber.

80 My invention furnishes a means of 85 smoothing and hardening the wood fiber, without diminishing its strength by the admixture of the harder fiber of straw.

85 Straw fiber possesses a fiber of hard, dense character but too short to be used for making strong paper, and I have found that by combining such straw cellulose with the long fiber of wood cellulose, the straw cellulose in a peculiar manner is greatly strengthened while the wood cellulose is rendered harder 90 and smoother, thus producing composite fiber which possesses a greater strength than the straw cellulose, and a greater smoothness and hardness than the wood cellulose.

95 My invention can be practiced by combining the cellulose from pine or other analogous wood with the cellulose made from rice, rye, wheat, or other straw.

An apparatus which may be employed to

practice this invention is shown in a dia-  
grammatic manner in the annexed drawing,  
A being the wood digester, B the straw di-  
gestor and C the blow-tank.

5 D is a manhole upon the wood digester to  
introduce the wood and the chemicals re-  
quired for reducing the same.

E is a pipe supplying steam of suitable  
temperature and pressure to the digester A;  
10 I a blow-off cock at the bottom of the di-  
gestor A, and M a pipe connecting such cock  
with the blow-tank.

D' is a manhole upon the straw digester  
to introduce the straw and chemicals re-  
quired for reducing the same; F' the pipe  
15 supplying the steam to such digester to cook  
the straw, the waste steam from the digester  
A being used in practice.

I' is the draw-off cock at the bottom of the  
20 digester B, and M' a pipe connecting the  
cock I' with the blow-tank C.

The pipes M and M' discharge pulp, in  
practice, into a baffle-tank C' within the blow-  
25 tank so that it is thoroughly disintegrated  
and mingled; and wash-pans J are shown be-  
neath the blow-tank into which the contents  
of the tank are discharged by a movable noz-  
zle N. A receptacle J is shown below the  
30 wash-pans J to receive the fiber when  
washed. The worm-wheels of the blow-off  
cocks I, I', are connected by a shaft K, and  
a shaft having a hand-wheel K' is connected  
therewith by bevel-gears L so that an opera-  
35 tor can empty both of the digesters simul-  
taneously into the blow-tank.

The materials are introduced into the re-  
spective digesters and treated in such a man-  
ner that the reduction of both to fiber is con-  
cluded at the same time, and the blow-off  
40 cocks I, I', are then simultaneously opened  
and the products of both digesters are dis-  
charged together into the blow-tank. The  
blow-tank is commonly open at the top.  
The two fibers are discharged from the di-  
45 gesters under such pressure and velocity that  
they are thoroughly disintegrated and inti-  
mately mingled with one another, and are  
so thoroughly amalgamated as to produce a  
homogeneous substance possessing the qual-  
50 ities of both fibers and having different char-  
acteristics from any fiber heretofore known.  
Such result is produced by the disruption of  
the tissues in contact with one another, in a  
heated and consequently soft condition, by  
55 the expansion of the steam, and the explo-  
sive nature of the discharge; which mingles  
the wood and straw cellulose together when  
discharged simultaneously from separate di-  
gesters.

60 The presence of the reducing liquor dur-  
ing such intermingling of the tissues also  
has a solvent effect upon the cellulose in the  
wood and straw, and unites them in a more  
perfect manner than is possible after they  
65 have been washed or bleached, or subjected

to any refining process which would shorten  
them or diminish their capacity for such  
union.

The product claimed herein is an un-  
bleached composite fiber in which the long  
70 fiber of wood and the short fiber of straw  
are intimately mingled without any mechan-  
ical treatment and so effectively combined  
that they will not separate when properly  
treated for use in making paper upon a  
75 paper machine. This composite fiber is  
readily distinguished by its color from any  
mixture of previously manufactured or  
bleached fibers. This duplex or composite  
80 fiber is capable of making a dense, strong,  
high-grade paper, and can be used without  
treating it injuriously in a beating engine,  
and its method of manufacture therefore  
avoids injury to the wood fiber while it  
85 saves expense and labor in its preparation.  
The composite fiber may thus be prepared  
for use in making high-grade papers, with-  
out impairing the strength of the fiber. The  
means for making this composite fiber by  
90 reduction of the two materials separately  
and blowing the products together, under  
pressure, is not claimed herein; but is made  
the subject of a separate application. No.  
375,568 filed May 25, 1907.

Having thus set forth the nature of the  
invention what is claimed herein is:

1. The process of making a composite  
fiber of wood cellulose and straw cellulose,  
which consists in simultaneously but sepa-  
rately reducing the wood to produce wood  
cellulose and the straw to produce straw  
cellulose, and then mingling the wood cellu-  
lose with the straw cellulose while in a heat-  
ed condition and mixed with the reducing  
liquor.

2. The process of making a composite  
fiber of wood cellulose and straw cellulose,  
which consists first, in reducing the wood  
and straw to fiber with chemical liquor si-  
multaneously by separate treatments, and  
second, simultaneously discharging the two  
fibers with the chemical liquor under pres-  
sure into contact with one another to dis-  
integrate them and unite them into a composite  
fiber.

3. The process of making a composite  
fiber of wood cellulose and straw cellulose,  
which consists first, in reducing the wood  
and straw to fiber with chemical liquor si-  
multaneously by separate treatments, and  
second, simultaneously disintegrating the  
two fibers in contact with one another to  
mingle and amalgamate them thoroughly.

In testimony whereof I have hereunto set  
my hand in the presence of two subscribing  
witnesses.

PULASKI M. HAMLIN.  
Witnesses:

JESSIE G. VANDINE,  
ELIZABETH DE HART.